

Patented Dec. 15, 1925.

1,565,323

# UNITED STATES PATENT OFFICE.

HARRY C. HAAK, OF SCRANTON, PENNSYLVANIA.

METHOD OF COOLING INTERNAL-COMBUSTION ENGINES.

No Drawing.

Application filed January 7, 1922. Serial No. 527,721.

To all whom it may concern:

Be it known that I, HARRY C. HAAK, a citizen of the United States, residing in Scranton, in the county of Lackawanna and 5 State of Pennsylvania, have invented certain new and useful Improvements in Methods of Cooling Internal-Combustion Engines, whereof the following is a specification.

10 My invention relates to the cooling of internal combustion engines, and especially to the cooling medium employed. An important object of my invention is to obviate ill effects of cold weather on an automobile, 15 motor boat, and other such internal combustion engines, and especially to do away with the risk of injurious freezing up of the engine. Still other advantages that can be secured through my invention will become 20 apparent hereinafter. Contrary to what is naturally to be expected from the deleterious and dangerous effects of lubricating oil when it finds its way into steam boilers, I have discovered that liquid hydrocarbons 25 possessing certain characteristics (such as hereinafter indicated) can be safely and very successfully used to cool the cylinders of internal combustion engines by circulation back and forth through the cylinder 30 jacket and the radiator, just as water is commonly used for that purpose.

To be used successfully and to the best advantage for the purposes of my invention, such media as just indicated must, in the 35 first place, be exempt from freezing, congealing, or great viscosity until quite low temperatures are reached: i. e., in general, temperatures approaching or ranging downward from zero Fahrenheit. Otherwise, the 40 medium would be liable to freeze when an automobile was left standing in cold weather, and either disrupt the radiator, cylinder jackets, or other parts of the cooling system at once, or else block the circulating 45 pump, etc., and cause trouble when the engine was started again. On the other hand, the medium must be unaffected by fairly high temperatures, approaching or exceeding the boiling point of water. If it boils 50 at too low a temperature, it may boil away and leave the engine to overheat; or, if its flash point or its ignition point is too low, its use will be attended with excessive fire hazard. In general, the flash point and ignition point should not fall greatly below 55 some 250° F., and should preferably approxi-

mate 275°-300° F., or upward, and the boiling point should be materially higher. Again, the medium should be of relatively low volatility and vapor tension at temperatures below its boiling point, to minimize loss by evaporation in service and risk of fire or explosion. For the latter reasons, it should likewise be relatively (if not absolutely) uninflammable. At service temperatures generally, of course, the medium must be of such relatively low viscosity that it can be circulated through the cooling system without undue resistance and expenditure of power. Unduly high viscosity is also disadvantageous because it rather tends toward burning or carbonization of the medium if the same becomes overheated in the system.

Indifference to fairly high temperatures is of the more importance, because most liquids otherwise suitable have a specific heat lower than that of water, and hence absorb relatively less heat than water for a given rise in temperature. With suitable indifference to fairly high temperatures, however, a hydrocarbonaceous medium will in use retain heat better and longer than water, since it will stand heating to a higher temperature. This means that when left standing the engine will remain warm longer, and is, therefore, more easily started after standing a short time. Also, the engine will run more smoothly on account of the more uniform temperature maintained by my more heat retentive cooling medium.

Mineral oils of the high boiling character indicated above are generally very well suited for the purpose of my invention, and particularly petroleum distillates. Such a cooling medium may have a specific gravity 95 ranging from about .860 (32 Baumé) to about .910 (24 Baumé). The relative uninflammability which such oils naturally display may be enhanced to a degree of virtual immunity, if desired, by admixture of an anti-inflammatory agent, such as carbon tetrachloride, or non-inflammable oils. Ordinarily, a minor admixture (some 5-15%) of carbon tetrachloride,—insufficient to affect (raise) the freezing point of the medium 100 materially,—will render such a medium sufficiently uninflammable for all practical needs. A relatively thin, non-viscous agent like carbon tetrachloride is also beneficial in diminishing the viscosity of the medium at 110 very low temperatures.

Especially suitable for the purpose is the

higher boiling kerosene fraction or series of petroleum. Petroleum kerosenes in general have boiling point ranging from about 300° F., to 570° F.; but I prefer the higher boiling kerosenes,—about 500° F., and upward. What is commercially known as "2-300 Miners 80" is such a kerosene. Ordinarily, I prefer to "compound" the kerosene employed somewhat, by intermixture 10 with non-inflammable oil of correspondingly high boiling point belonging to the lubricating series or fraction of petroleum, preferably those of pour test —30° F., to —40° F. Usually this is done in order to 15 thicken the kerosene; but in some cases, it may be desirable to thin it by compounding. Petroleum lubricating oils in general have boiling points ranging from 570° to 750° F.,—sometimes as low as 400° F. For reasons 20 which will appear hereinafter, it is preferable that the boiling point of the lubricating oil used should not greatly exceed that of the kerosene, but rather be about the same. The proportions of kerosene and lubricating oil to be employed depend both on the properties of the particular grades actually used and on the conditions of the service for which the product is intended. Using "No. 2-300 Miners 80" 25 kerosene, it is an easy matter, with the aid of an hydrometer, to add and mix in, little by little, the right amount of lubricating oil of corresponding boiling point to bring the aggregate to an appropriate low degree of 30 viscosity within the range of specific gravities indicated above. I have found it advantageous to make the mixture in "heavy", "medium", and "light" grades,—ranging from zero F., to 30° below in freezing point, 35 according to specific gravity,—for use under different climatic and temperature conditions. With the above mentioned "No. 2-300 Miners 80", the composite medium should easily give a flash test of 300° F., and a fire (or ignition) test of 340° F. Carbon tetrachloride may be added to the 40 primary mixture in the proportion of from 10 to 12½% of the final product without thinning it unduly or injuriously affecting 45 the freezing point.

Besides possessing the properties and advantages already indicated, this product is of low viscosity; volatilizes so slowly in service that one filling of the cooling system of an automobile will usually last all 50 winter; is initially non-inflammable, and is not rendered materially inflammable by the progressive changes induced in it by heating in normal service; can be safely charged or recharged into the cooling system even 55 while the engine is running; and is less costly than the alcohol and glycerine admixture sometimes used with water to pre-

vent freezing, besides being more permanent.

(Both alcohol and glycerine evaporate off faster than the water, so that the mixture changes in composition and must be constantly watched and the anti-freezing addition renewed from time to time; and glycerine tends to congeal to a gelatinous mass which impedes circulation, and decomposes to "acrolein" with a tendency to increase rust and incrustation.) Also, the product 65 cleans and frees the radiator and water jacket from rust, and so increases their life 70 and obviates incrustation and corrosion. When the main ingredients above described (kerosene and lubricating oil) are of about 75 the same boiling point, the mixture remains substantially homogeneous and constant as regards its more important properties, and does not burn or carbonize, or give rise to 80 carbonaceous or other solid deposits of any sort in the cooling system. If the medium 85 were not fairly homogeneous, but, on the contrary, comprised hydrocarbons of widely different boiling points and viscosity, the thin lower boiling portions would tend to 90 evaporate off whenever the engine became somewhat overheated, so that eventually the medium might become so thick or overviscid as to carbonize in the cylinder jackets as a result of too sluggish circulation.

Having thus described my invention, I 95 claim:

1. The method of cooling an internal combustion engine which consists in circulating a frigorific medium thereabout composed of a high boiling mineral oil including a minor quantity of carbon tetrachloride varying from 5 to 15% of the final 100 product.

2. The method of cooling an internal combustion engine which consists in circulating 105 a frigorific medium through the cylinder jackets and radiator composed of a high boiling kerosene fraction of petroleum with a minor quantity of tetrachloride in proportion varying from 10 to 12.5% of the 110 final product.

3. A cooling medium for circulation about the cylinder jackets and through the radiator of internal combustion engines comprising an admixture of high boiling 115 petroleum kerosene with a flash point approaching 300 degrees F. and upward; with a freezing point ranging downward from zero F.; of specific gravity about .85 to .91; and carbon tetrachloride in proportion varying from 5 to 15% of the final product.

In testimony whereof, I have hereunto signed my name at Philadelphia, Pennsylvania, this 5th day of January, 1922.

HARRY C. HAAK.